

Nov. 5, 1974

G. J. REINIS

3,846,127

IMAGING SYSTEM

Filed Aug. 30, 1972



**1**

3,846,127

**IMAGING SYSTEM**

Gedeminas J. Reinis, Rochester, N.Y., assignor to  
Xerox Corporation, Stamford, Conn.  
Filed Aug. 30, 1972, Ser. No. 284,817

Int. Cl. G03c 5/10

U.S. CL. 96—1 M

23 Claims

**ABSTRACT OF THE DISCLOSURE**

In an imaging system wherein a cohesively weak photo-responsive imaging layer comprising photosensitive pigment particles dispersed in an insulating binder is sandwiched between two sheets, then exposed to a pattern of actinic electromagnetic radiation and an electric field thereby providing upon separation of the sheets a positive image on one sheet and a negative image on the other, the electrically photosensitive pigment particles are treated with polyisobutylene succinic anhydride or derivatives thereof before being incorporated in the imaging layer thus resulting in improved images.

**BACKGROUND OF THE INVENTION**

The present invention relates in general to imaging and more specifically to an imaging method for the formation of images by imaging layer transfer in image configuration as well as the imaging materials used therein.

Manifold imaging, a technique based on layer transfer of a colored material in image configuration is described in detail in copending application Ser. No. 708,380, filed Feb. 26, 1968, and incorporated by reference herein. Generally speaking, manifold imaging utilizes a structure comprising an electrically photosensitive cohesively weak (or field fracturable) imaging layer sandwiched between a donor sheet and a receiving sheet. An electric field is imposed across the imaging layer and the imaging layer is exposed to imagewise actinic radiation. Upon separation of the donor and receiver sheets the imaging layer fractures in imagewise configuration corresponding to the image-wise exposure with an image which is positive in image sense adhering to one of the sheets and an image which is negative in image sense adhering to the other sheet. Although imaging layers may be prepared which are themselves cohesively weak or field fracturable to respond to the application of light and electric field, a larger range of materials may be used if an "activating" step is included in the process. The activating step serves to structurally weaken the imaging layer so that it can be more easily fractured along a sharp line which defines the image to be reproduced. Conventionally the imaging layer is activated by treating it with a swelling agent or a partial solvent for the material prior to placing the imaging layer between the donor and the receiver sheets. Alternatively, the activating step may be omitted if, for example, the layer retains sufficient residual solvent after having been coated on a substrate from a solution or paste to render the layer cohesively weak.

Manifold imaging has been found to be capable of producing images of excellent quality. The imaging system, in order to achieve the optimum resolution and color separation that it is capable of producing, requires photoconductive pigment particles which are as small as possible and which preferably remain as individual species during the entire process of imaging layer formation and imaging. Moreover the commercial utilization of the process involves relatively long term storage of the imaging layer compositions thus necessitating stable imaging compositions. It would be desirable to have photosensitive pigment particles which remain as individual species during the process of imaging layer formation and imaging as well as providing imaging compositions which are stable over relatively long periods of time.

**2**

The present invention relates to a novel treatment for the photoconductive pigment particles incorporated in the imaging layer as well as the resulting photoconductive pigment particles obtained from such treatment.

**SUMMARY OF THE INVENTION**

It is, therefore, an object of this invention to provide a manifold imaging system having the above-described desirable features.

It is another object of the invention to provide a treatment for photoconductive pigment particles employed in the imaging layer of the manifold imaging process.

It is still another object of the invention to provide novel photoconductive pigment particles for use in the imaging layers of the manifold imaging process.

It is a further object of the invention to provide imaging compositions which are stable over relatively long periods of time for use in the manifold imaging process.

The above-described and other objects and advantages are realized in accordance with the present invention by treating the electrically photosensitive pigment particles with a polyisobutylene succinic anhydride derivative prior to incorporating the particles in an insulating binder material to form the imaging layer composition used in the manifold imaging process. The compounds used for the treatment of the electrically photosensitive pigment particles include polyisobutylene succinic anhydride and reaction products of polyisobutylene succinic anhydride with various compounds having polar groups such as, for example,

water, primary amines, secondary amines, polyhydric alcohols, inorganic metal hydroxides and the like.

The invention will be more fully understood from the following detailed description of various preferred embodiments thereof particularly when read in conjunction with the accompanying drawing wherein the Figure is a side sectional view of a typical photosensitive imaging manifold set.

Referring now to the Figure there is seen a supporting donor substrate layer 11 and an imaging layer generally designated 12. In the manufacture of the imaging member, herein referred to as the manifold set, layer 12 is preferably coated on substrate 11 so that it adheres thereto. These layers are collectively referred to as the imaging donor or merely the donor. In this particular illustrative

example, layer 12 comprises photoconductive pigment particles 13 dispersed in a binder 14. Above imaging layer 12 is a third or receiving layer 16. This receiver sheet is ordinarily supplied as a separate layer which does not initially adhere to layer 12. Accordingly, although the

whole imaging member or "manifold set" may be supplied in a convenient three-layer sandwich as has been illustrated, receiving layer 16 may also be supplied as a separate sheet or roll if desired. On the other hand, in those systems where activation of the imaging layer is not required or where imaging layer 12 has been preactivated, layer 16 may adhere to or be tacked onto imaging layer 12.

In the particular embodiment of the manifold set shown in the Figure both the donor substrate 11 and the receiver sheet 16 are made up of an electrically conductive material such as cellophane with at least one of them being optically transparent to provide for the exposure of layer 12. In this embodiment of the manifold set layers 11 and 16 also act as the electrodes.

The imaging layer may contain any suitable electrically photosensitive material. Typical organic materials include: quinacridones such as: 2,9-dimethyl quinacridone, 4,11-dimethyl quinacridone, 2,10-dichloro-6,13-dihydro-quinacridone, 2,9-dimethoxy-6,13-dihydro-quinacridone, 2,4,9,11-tetrachloroquinacridone, and solid solutions of quinacridones and other compositions as described in U.S. Pat. 3,160,510; carboxamides such as: N-2'-pyridyl-8,13-dioxodinaphtho-(2,1-2,3)-furan-6-carboxamide, N-2'-

(1'',3''-diazyl)-8,13-dioxodinaphtho-(2,1-2',3')-furan - 6-carboxamide, anthra-(2,1,8)-naphtho-(2,3-d)-furan-9,14-dione-7-(2'-methyl-phenyl)-carboxamide; carboxanilides such as: 8,13-dioxodinaphtho-(2,1-2',3')-furan-6-carbox-p-methoxy-anilide, 8,13-dioxodinaphtho-(2,1-2',3')-furan-6-carbox-m-chloroanilide, 8,13-dioxodinaphtho-(2,1-2',3')-furan-6-carbox-p-cyanoanilide; triazines such as: 2,4-diamino - triazine, 2,4 - di(1' - anthraquinonyl-amino)-6-(1''-pyrenyl)-triazine, 2,4-di(1' - anthraquinonyl-amino)-6-(1''-naphthyl)-triazine, 2,4-di(1' - naphthyl-amino)-6-(1'-perylene)-triazine, 2,4,6 - tri - (1',1',1'''-pyrenyl)-triazine; benzopyrrocolines such as: 2,3-phthaloyl-7,8-benzopyrrocoline, 1-cyano-2,3 - phthaloyl - 7,8-benzopyrrocoline, 1-cyano-2,3-phthaloyl-5 - nitro - 7,8-benzopyrrocoline; 1-cyano-2,3-phthaloyl-5-acetamido-7,8-benzopyrrocoline; anthraquinones such as: 1,5-bis-(beta-phenylethylamino) anthraquinone, 1,5-bis-(3'-methoxy-propylamino) anthraquinone, 1,5-bis (benzylamino) anthraquinone, 1,5-bis (phenylbutylamino) anthraquinone, 1,2,5,6 - di(C,C'-diphenyl)-thiazole-anthraquinone, 4-(2'-hydroxyphenyl-methoxyamino) anthraquinone; azo compounds such as: 2,4,6-tris(N-ethyl-N-hydroxy-ethyl-p-aminophenylazo) phloroglucinol, 1,3,5,7-tetrahydroxy-2,4,6,8-tetra (N-methyl-N-hydroxy-ethyl-p-amino-phenyl-azo) naphthalene, 1,3,5-trihydroxy-2,4,6-tri (3'-nitro-N-methyl-N-hydroxymethyl-4'-aminophenylazo) benzene, 3-methyl-1-phenyl-4-(3'-pyrenylazo)-2-pyrazolin-5-one, 1-(3'-pyrenylazo)-2-hydroxy-3-naphthanilide, 1-(3'-pyrenyl-azo)-2-naphthol, 1-(3'-pyrenylazo)-2-hydroxypyrene, 1-(3'-pyrenylazo)-2-hydroxy-3-methyl-xanthene, 2,4,6-tris (3'-pyrenylazo) phloroglucinol, 2,4,6-tris (1'-phenanthrenylazo) phloroglucinol, 1-(2'-methoxy-5'-nitrophenyl-azo)-2-hydroxy-3''-nitro-3-naphthanilide; salts and lakes of compounds derived from 9-phenylxanthene, such as: phosphotungstomolybdic lake of 3,6-bis (ethylamino)-9,2'-carboxyphenyl xanthronium chloride, barium salt of 3,2'-toluidine amino-6,2'-methyl-4''-sulphophenyl-amino-9,2'-carboxyphenyl xanthene; phosphomolybdic lake of 3,6-bis (ethylamino)-2,7-dimethyl-9,2'-carbethoxy-phenyl-xanthenonium chloride; dioxazines such as: 2,9-dibenzoyl-6,13-dichloro-triphenodioxazine, 2,9-diacetyl - 6,13 - di-chloro-triphenodioxazine, 3,10-dibenzoylamine-2,9-diisopropoxy-6,13-dichloro-triphenodioxazine, 2,9-difuroyl - 6,13-dichloro-triphenodioxazine; lakes of fluorescein dyes such as: lead lake of 2,7-dinitro-4,5-dibromo fluorescein, lead lake of 2,4,5,7-tetrabromo fluorescein, aluminum lake of 2,4,5,7-tetrabromo-10,11,12,13-tetrachloro fluorescein; bisazo compositions such as: N,N'-di [1-(1'-naphylazo)-2-hydroxy-8-naphthyl] adipamide, N,N'-di-1-(1'-naphthylazo)-2-hydroxy-8-naphthyl succindiamide, bis-4,4'-(2''-hydroxy-8''-N,N'-diterephthalamide-1 - naphthylazo) biphenyl, 3,3'-methoxy-4,4'-diphenyl-bis(1'-azo-2''-hydroxy-3''-naphthanilide); pyrenes such as: 1,3,6,8-tetracyanopyrene, 1,3-dicyano-6,8-dibromo-pyrene, 1,3,6,8-tetraaminopyrene, 1-cyano-6-nitropyrene; phthalocyanines such as: beta-form metal-free phthalocyanine, copper phthalocyanine, tetrachloro phthalocyanine, the "x"-form of metal-free phthalocyanine as described in U.S. Pat. 3,357,989; metal salts and lakes of azo dyes, such as: calcium lake of 6-bromo-1-(1'-sulfo-2-naphthylazo)-2-naphthol, barium salt of 6-cyano-1-(1'-sulfo-2-naphthylazo)-2-naphthol, calcium lake of 1-(2'-azonaphthalene-1'-sulfonic acid)-2-naphthol, calcium lake of 1-(4'-ethyl-5'-chloroazobenzene-2'-sulfonic acid)-2-hydroxy - 3 - naphthoic acid; and mixtures thereof.

Typical inorganic compositions include cadmium sulfide, cadmium sulfoselenide, zinc oxide, zinc sulfide, sulphur, selenium, mercuric sulfide, lead oxide, lead sulfide, cadmium selenide, titanium dioxide, indium trioxide and the like.

In addition to the aforementioned organic materials other organic materials which may be employed in the imaging layer include:

polyvinylcarbazole; 2,4-bis-(4,4'-diethyl-amino-phenyl)-1,3,4-oxidiazole; N-isopropylcarbazole; polyvinylanthracene; triphenylpyrrol; 4,5-diphenylimidazolidinone; 4,5-diphenylimidazolidinethione; 4,5-bis-(4-amino-phenyl)-imidazolidinone; 1,2,5,6-tetraazacyclooctatetraene-(2,4,6,8); 3,4-di-(4'-methoxyphenyl)-7,8-diphenyl-1,2,5,6-tetraaza-cyclooctatetraene-(2,4,6,8); 3,4-di-(4'-phenoxyphenyl)-7,8-diphenyl-1,2,5,6-tetraaza-cyclooctatetraene-(2,4,6,8); 3,4,7,8-tetramethoxy-1,2,5,6-tetraaza-cyclooctatetraene-(2,4,6,8); 2-mercaptop-benzthiazole; 2-phenyl-4-alpha-naphthylidene-oxazolone; 2-phenyl-4-diphenylidene-oxazolone; 2-phenyl-4-diphenylidene-oxazolone-2-phenyl-4-p-methoxy-benzylidene-oxazolone; 6-hydroxy-2-phenyl (p-dimethyl-amino phenyl)-benzofurane; 6-hydroxy-2,3-di(p-methoxyphenyl)benzofurane; 2,3,5,6-tetra-(p-methoxy-phenyl)-furo-(3,2f)-benzofurane; 4-dimethyl-amino-benzylidene-benzhydrazide; 4-dimethyl-aminobenzylidene-iso-nicotinic acid hydrazide; furfurylidene-(2)-4'-dimethylamino-benzhydrazide; 5-benzylidene-amino-acenaphthene-3-benzylidene-amino-carbazole; (4-N,N-dimethylamino-benzylidene)-p-N,N-dimethyl-aminoaniline; (2-nitrobenzylidene)-p-bromo-aniline; N,N-dimethyl-N'-(2'-nitro-4-cyano-benzylidene)-p-phenylene-diamine; 2,4-diphenyl-quinazoline; 2-(4'-amino-phenyl)-4-phenyl-quinazoline; 2-phenyl-4-(4'-dimethyl-amino-phenyl)-7-methoxy-quinazoline; 1,3-diphenyl-tetra-hydroimidazole; 1,3-di-(4'-chlorophenyl)-tetra-hydroimidazole; 1,3-diphenyl-2,4'-dimethylaminophenyl)-tetra-hydroimidazole; 1,3-di-(p-tolyl)-2-[quinolyl-(2')]tetra-hydroimidazole; 3-(4'-dimethylamino-phenyl)-5-(4''-methoxy-phenyl)-6-phenyl-1,2,4-triazine; 3-pyridyl-(4')-5-(4'-dimethylamino-phenyl)-6-phenyl-1,2,4-triazine; 3-(4'-amino-phenyl)-5,6-di-phenyl-1,2,4-triazine; 2,5-bis [4'-amino-phenyl-(1')]1,3,3-triazole; 2,5-bis [4'-(N-ethyl-N-acetyl-amino)-phenyl)-1']1,3,4-triazole; 1,5-diphenyl-3-methyl-pyrazoline; 1,3,4,5-tetra-phenyl-pyrazoline; 1-phenyl-3-(p-methoxy styrl)-5-(p-methoxy-phenyl)-pyrazoline; 1-methyl-2-(3',4'-dihydroxy-methylene-phenyl)-benzimidazole; 2-(4'-dimethylamine phenyl)-benzoxazole; 2-(4'-methoxyphenyl)-benzthiazole; 2,5-bis [p-amino-phenyl-(1)]1,3,4-oxidiazole; 4,5-diphenyl-imidazolones; 3-amino-carbazole; copolymers and mixtures thereof.

Other materials include organic donor-acceptor (Lewis acid-Lewis base) charge-transfer complexes made up of aromatic donor resins such as phenolaldehyde resins, phenoxides, epoxides, polycarbonates, urethanes, styrene or the like complexed with electron acceptors such as: 2,4,7-trinitro-9-fluorenone; 2,4,5,7-tetranitro-9-fluorenone; picric acid; 1,3,5-trinitro benzene; chloranil, 2,5-dichloro-benzoquinone; anthraquinone-2-carboxylic acid, 4-nitro-phenol; maleic anhydride; metal halides of the metals and metalloids of groups I-B and II-VIII of the Periodic table including for example, aluminum chloride,

zinc chloride, ferric chloride, magnesium chloride, calcium iodide, strontium bromide, chromic bromide, arsenic triiodide, magnesium bromide, stannous chloride etc.; boron halides, such as boron trifluorides; ketones such as benzophenone and anisil, mineral acids such as sulfuric acid; organic carboxylic acids such as acetic acid and maleic acid, succinic acid, citroconic acid, sulphonic acid, such as 4-toluene sulphonic acid and mixtures thereof. In addition to the charge transfer complexes, it is to be noted that many other of the above materials may be further sensitized by the charge transfer complexing technique and that many of these materials may be dye-sensitized to narrow, broaden or heighten their spectral response curves.

It is also to be understood in connection with the heterogeneous system, that the photoconductive particles themselves may consist of any suitable one or more of the aforementioned photoconductors, either organic or inorganic dispersed in, in solid solution in, or copolymerized with, any suitable insulating resin whether or not the resin itself is photoconductive. This particular type of particle may be particularly desirable to facilitate dispersion of the particle to prevent undesirable reactions between the binder 14 and the photoconductor or between the photoconductor and the activator and for similar purposes. Typical resins of this type include polyethylene, polypropylene, polyamides, polymethacrylates, polyacrylates, polyvinyl chlorides, polyvinyl acetates, polystyrene, polysiloxanes, chlorinated rubbers, polyacrylonitrile, epoxies, phenolics, hydrocarbon resins and other natural resins such as rosin derivatives as well as mixtures and copolymers thereof.

Generally the materials used for the treatment of the electrically photosensitive pigment particles are obtained as the reaction products of polyisobutylene succinic anhydride with any suitable compound having polar groups.

The polyisobutylene succinic anhydride used in accordance with this invention may be obtained from several commercial sources or may be prepared as below. It is suitable to use polyisobutylene having a number average molecular weight up to about 10,000, with a preferred range being up to about 5,000.

#### Preparation of Polyisobutylene succinic

In a five liter four-necked round bottom flask place 2,000 gm. of polyisobutylene (Oronite Polybutene 24, number average molecular weight 950, from California Chemical Co., Oronite Division), and 200 gm. maleic anhydride. A thermometer, oil-sealed stirrer, a wide air condenser, and a gas inlet tube are attached, one to each of the flask necks, with Teflon-covered ground glass joints. A slight positive flow of dry purified nitrogen is introduced through the gas inlet tube. By use of a heating mantle the temperature of the flask's contents is raised to 200° C. and maintained for 24 hours with stirring. Then the flask contents are allowed to cool and dissolved in three liters of cyclohexane. The contents (solution) is filtered through a Johns-Manville Celite filter-aid to remove unreacted and undissolved maleic anhydride. The filtrate is then placed, piecemeal, in a three liter, three-neck vacuum distillation flask. The cyclohexane is distilled off at about 70° C. and then the temperature is raised slowly (with stirring) to 200° C. at about 10 Torr to remove unreacted but dissolved maleic anhydride and hydrocarbon "light-ends." The viscous polyisobutylene succinic anhydride is cooled, poured into suitable wide mouth containers and stored until use.

Suitable polar agents which may be reacted with polyisobutylene succinic anhydride to obtain derivatives of the anhydride suitable for use in accordance with this invention are: water, primary amines, secondary amines, polyhydric alcohols, inorganic metal hydroxides and the like, which yield the corresponding acid, amide or imide, ester and metal salt of polyisobutylene succinic anhydride. Usually the derivative number average molecular weight is

in the range up to about 10,000 with the preferred range being up to about 5,000.

#### Polyisobutylene succinic Acid

5 The conversion of polyisobutylene succinic anhydride to polyisobutylene succinic acid is accomplished by the well known method of hydrolyzing the anhydride by the addition of water in an acidic medium. A pH of from about 1 to about 4 is the preferred acidic range.

10 **Polyisobutylene succinamide**  
15 Typical suitable primary or secondary amines having a primary or secondary amino group include: lower aliphatic amines such as methylamine, dimethylamine, ethylamine, diethylamine, n-propylamine, dipropylamine, isopropylamine, diisopropylamine, allylamine, diallylamine, n-butyramine, dibutylamine, isobutylamine (2-methylpropylamine), diisobutylamine, etc.; higher aliphatic (fatty) amines such as decylamine, dodecylamine, tetradecylamine, hexadecylamine, tetraethylene pentamine, octadecylamine, etc.; and aromatic amines such as benzylamine,  $\beta$ -phenylethylamine, etc. The reaction entails simply heating and mixing a mole to mole mixture of the amine and anhydride.

#### Polyisobutylene succinimide

20 The conversion of polyisobutylene succinic anhydride to a polyisobutylene succinimide is accomplished by established aminolysis reactions, followed by heating. Generally, it is preferred to react the amines with the anhydride during the application of heat wherein the temperature is maintained from about 180° C. to about 210° C. Although the reacting amine should contain a primary amine, the resulting polyisobutylene succinimide may also contain the primary, secondary or tertiary amines or mixtures thereof. A particularly preferred polyisobutylene succinimide results upon the reaction of polyisobutylene succinic anhydride with an amine having the general formula  $\text{NH}_2-(\text{CH}_2-\text{CH}_2-\text{NH})_x-\text{CH}_2-\text{CH}_2-\text{NH}_2$  at about 200° C. wherein  $x$  is from 0 to 10; such as tetraethylene pentamine where  $x=3$  above.

#### Ester of Polyisobutylene succinic Acid

25 The term "polyhydric alcohol" is used herein to refer to alcohols having two or more hydroxyl groups. Typical suitable polyhydric alcohols include, ethylene glycol; 1,2 propanediol; pentaerythritol (2,2-bis (hydroxymethyl)-1,3-propanediol); dipentaerythritol; tripentaerythritol; trimethylolethane (2-hydroxymethyl-2-methyl-1,3-propanediol); trimethylopropane (2-ethyl-2-hydroxymethyl-1,3-propanediol); 1,2,4-butanetriol (1,2,4-trihydroxybutane); 1,2,6-hexanetriol (1,2,6-trihydroxylethane); anhydroneahaepitol tetrahydro-3,3,5,5-tetrakis (hydroxymethyl)-4-pyranol.

30 These and other suitable alcohols may be utilized in the esterification of polyisobutylene succinic acid from the anhydride. The esterification is usually carried out at a temperature above about 80° C., normally between 100° C. and 150° C. Catalysts such as phosphoric acid, sulfuric acid, pyridine hydrochloride, p-toluene sulfonic acid and other suitable esterification catalysts may be used, normally in an amount from about 0.01% to about 0.05% of the reaction mixture weight.

#### Metal Salt of Polyisobutylene succinic Acid

35 Typical suitable inorganic metal hydroxides include the hydroxides of zinc, cadmium, lead, calcium, manganese and cobalt. Zinc and cadmium hydroxides are preferred for giving enhanced results when used in accordance with the practice of this invention. The conversion of polyisobutylene succinic anhydride into a metal salt of polyisobutylene succinic acid may be accomplished by reacting the anhydride, water and metal salt while maintaining a temperature of about 100° C. One mole of the anhydride is

reacted with from 0.5 to 4.0 moles of the metal hydroxide; with 1 to 2 moles of the hydroxide preferred.

The relative proportions of the polyisobutylene succinic anhydride and the suitable polar agents which are to be used depend upon the product characteristics desired. For purposes of the practice of this invention, a number average molecular weight for the polyisobutylene succinic anhydride and its equivalents derived from its reaction with suitable polar agents, of up to about 10,000 is satisfactory; of up to about 5,000 being preferred. Generally, from about 20% to about 200% by weight of treating agent based on the weight of photosensitive pigment particles is employed.

Two general methods of treatment have been found effective in reducing background. Both methods involve intimate contact, such as ball milling, the photosensitive pigments with polyisobutylene succinic anhydride or derivatives thereof. In the first method, followed in Example I below, most of the anhydride or derivative is carried away by the vacuum filtering. Although it is not known why the practice of this invention provides the result of low background imaging, nor how the anhydride or derivatives operate within the imaging system, it is believed that small quantities of the anhydride or derivatives modify the surface of the pigments in each of the two general treatment methods.

The second general method is the same as the first except that the anhydride or derivatives are not removed from the mixture of pigment and the anhydride or derivatives and becomes incorporated in the binder matrix of the imaging layer. This results in the anhydride or derivatives being substantially uniformly dispersed in the binder of the imaging layer along with photosensitive pigments believed to have some of the anhydride or derivatives absorbed on their surfaces. This dispersion of treating agent aids in the fracture of a fracturable photo-responsive imaging layer, such as that of U.S. Pat. 3,615,393 hereby incorporated by reference.

As a general rule, it is preferable to use the higher portion of the previously recited 20% to 200% range by weight of treating agent (i.e., polyisobutylene succinic anhydride or its derivatives) based on the weight of photosensitive pigment particles, in the first treatment method above, and to use the lower portion of the range in the second treatment method just described. That is, from 20% to 110% for the second method and from 110% to 200% for the first method. This observance generally provides optimum imaging characteristics for the resulting imaging layer. However, any percentage in the range for either method improves low background imaging relative to untreated pigment particles and imaging layers.

The photosensitive pigment particles are typically treated with the polyisobutylene succinic anhydride or its derivatives of the invention by ball milling a dispersion of the pigment in a solution of the treating agent. It is preferred to use a poor solvent for the treating agent e.g. D.C. Naphtha, so that only a small amount will go into solution. Optionally another solvent such as isopropanol or the like may be added to reduce solubility.

The binder material in the heterogeneous imaging layer or the material used in conjunction with the photoresponsive material in the homogenous layer, where applicable, may comprise any suitable cohesively weak insulating material or materials which can be rendered cohesively weak. Typical materials include: microcrystalline waxes such as: Sunoco 1290, Sunoco 5825, Sunoco 985, all available from Sun Oil Co.; Parafin RG, available from the Moore and Munger Company; paraffin waxes such as: Sunoco 5512, Sunoco 3425, available from Sun Oil Co.; Sohio Parowax, available from Standard Oil of Ohio; waxes made from hydrogenated oils such as: Capitol City 1380 wax, available from Capitol City Products, Columbus, Ohio; Caster Wax L-2790, available from Baker Caster Oil Co.; Vitikote L-304, available from Duro Commodities; polyethylenes such as: Eastman

Opolene N-11, Eastman Opolene C-12, available from Eastman Chemical Products, Polyethylene DYJT, Polyethylene DYLT, Polyethylene DYNF, Polyethylene DYDT, all available from Union Carbide; Marlex TR 822, Marlex 1478, available from Phillips Petroleum Co.; Epolene C-13, Epolene C-10, available from Eastman Chemical Products, Polyethylene AC8, Polyethylene AC612, Polyethylene AC324, available from Allied Chemicals; modified styrenes such as: Piccotex 75, Piccotex 100, Piccotex 120, available from Pennsylvania Industrial Chemical; Vinylacetate-ethylene copolymers such as: Elvax Resin 210, Elvax Resin 310, Elvax Resin 420, available from Dupont; Vistanex MH, Vistanex L-80, available from Enjay Chemical Co.; vinyl chloride-vinyl acetate copolymers such as: Vinylite VYLF, available from Union Carbide; styrene-vinyl toluene copolymers; polypropylenes; and mixtures thereof. A mixture of microcrystalline and paraffinic waxes is preferred because it is cohesively weak and a good insulator.

As has been previously discussed the first step in the imaging process is the activation step when the latter is required. In this stage of the imaging process, the manifold set is opened and the activator is applied to imaging layer 12 following which these layers are closed back together again. The activator may be applied by any suitable technique such as with a brush, with a smooth or rough surfaced roller, by flow coating, by vapor condensation, by spraying or the like. The activator serves to swell or otherwise weaken and thereby lower the cohesive strength of imaging layer 12. The activator should preferably have a high level of resistivity to help prevent electrical breakdown of the manifold set.

Although it is preferred to use a separate electrode, sheet 16 for purposes of simplicity is shown as a conductive receiver sheet which also acts as an electrode. Potential source 28 is connected to resistor 30, receiver sheet 16 and substrate layer 11. An electrical field is applied across the manifold set and it is exposed to an image 29 to be reproduced. Upon separation of substrate 11 and receiving sheet 16, imaging layer 12 fractures along the edges of the exposed areas. Accordingly once separation is complete exposed portions of imaging layer 12 are retained on one or the other of layers 11 and 16 while unexposed portions are retained on the other layer, resulting in the formation of a high gamma positive image on one of the sheets and a high gamma negative image on the other.

The strength of the electrical potential applied across the manifold set depends on the structure of the manifold set and the materials used. For example, if highly insulating receiver and donor sheet materials are used, a much higher potential may be applied than if relatively conductive donor and receiver sheets are used. The field strength required may, however, be easily determined. If too large a potential is applied, electrical breakdown of the manifold set will occur allowing arcing across the manifold set. If too little potential is applied, the imaging layer will not fracture in imagewise configuration. By way of example, if a 3 mil Mylar (a polyester formed by the condensation reaction between ethylene glycol and terephthalic acid available from the E. I. du Pont de Nemours & Co., Inc.) receiver sheet and a 2 mil Mylar donor sheet are used, potentials as high as 20,000 volts may be applied between the electrodes. The preferred applied potentials across the manifold set are, however, in the range of from about 1,000 volts per mil to about 4,000 volts per mil. Since relatively high potentials are utilized, it is desirable to insert a resistor in the circuit to limit the flow of current. Resistors on the order of from 1 megohm to about 20,000 megohms are conventionally used.

A visible light source, an ultraviolet light source or any other suitable source of activating electromagnetic radiation may be used to expose the imaging layer of this invention. The electrically photosensitive material is

chosen so as to be responsive to the wavelength of the electromagnetic radiation used. It is to be noted that different photoresponsive materials have different spectral responses and that the spectral response of many photoresponsive materials may be modified by dye sensitization so as to either increase and narrow the spectral response of a material to a peak or to broaden it to make it more panchromatic in its response. Thus, the material can be used to make ordinary "black and white" images using panchromatic response while narrow spectral response materials may be employed for the production of color separations or the like. In addition, manifold images formed on transparent materials using different colored imaging layers such as cyan, magenta and yellow may be combined to produce full natural color images by superposition. Also, either the receiver or donor sheet may be opaque providing a print on one or the other sheet.

The manifold sets may be supplied in any color desired either by taking advantage of the natural color of the photoresponsive or binder materials in the imaging layer of the manifold set or by the use of additional dyes and pigments therein whether photoresponsive or not and, of course, various combinations of these photoresponsive and non-photoresponsive colorants may be used in the imaging layer so as to produce the desired color.

The invention will now be described in detail with respect to specific preferred embodiments by way of Examples it being understood that these are intended to be illustrative only and the invention is not limited to the procedures, conditions, materials, etc. recited therein. All parts and percentages listed are by weight unless otherwise specified.

#### EXAMPLE I

Pigments for a donor mixture are prepared as follows: 2.5 grams of Irgazin Red 2BLT pigment and 2.5 grams of Irgazin Yellow 2GLT pigment, both available from Geigy Chemical Co. and placed in a ball mill along with a solution of 1 gram of polyisobutylene succinimide of tetraethylene pentamine in petroleum ether and ball milled for about 20 hours at a temperature of from about 60-110° C. The resulting dispersion is vacuum filtered and then allowed to air dry.

A donor coating mixture is formulated according to the following procedure: 2 grams of x-form metal-free phthalocyanine pigment is ball milled in 50 ml. of petroleum ether at a temperature of 60-110° C. for about 20 hours. 3 grams of the above-mentioned treated red and yellow pigment mixture are dispersed in 50 ml. of petroleum ether at a temperature of 60-110° C. by means of an ultrasonic probe. The two dispersions are then mixed together and 5 grams of polyethylene designated as AG-612 and available from Allied Chemical Co. are dissolved in the dispersion by heating to 80° C. with moderate stirring. The dispersion is then quenched rapidly by adding 700 ml. of room temperature isopropyl alcohol. The precipitated mixture is then vacuum filtered and flushed with 200 ml. of isopropyl alcohol. The moist filter cake is redispersed in 100 ml. of isopropyl alcohol by means of an ultrasonic probe.

An approximately 25 $\mu$  thick coating of the donor mixture is applied to a Mylar sheet by means of a No. 22 Meyer drawdown rod and dried. After drying, the pigment binder layer is about 10 $\mu$  thick. The donor sheet thus formed is imaged in accordance with the manifold imaging procedure previously described. The images obtained are of moderate quality with low background on the receiver sheet and are superior to images made with no pretreatment of the red and yellow pigments.

#### EXAMPLE II

Example I is followed except that the pigments are ball milled with 2 grams of the polyisobutylene succinimide of tetraethylene pentamine.

#### EXAMPLE III

Example I is followed except that the pigments are ball milled with 3 grams of polyisobutylene succinimide.

#### EXAMPLE IV

Example I is followed with the exception that the pigments are ball milled with 5 grams of polyisobutylene succinimide.

#### EXAMPLES V AND VI

Example I is followed except that the pigments are ball milled with 3 grams of the zinc salt of polyisobutylene succinimide in Example V and 3 grams of the cadmium salt of polyisobutylene succinimide in Example VI.

#### EXAMPLE VII

Example I is followed with the exception that the pigments are ball milled with 10 grams of the ethylene glycol monoester of polyisobutylene succinimide (formed by reacting 1 mole of ethylene glycol with polyisobutylene succinimide).

Although specific components and proportions have been stated in the above description of preferred embodiments of the invention, other typical materials as listed above as suitable may be used with similar results. In addition, other materials may be added to the mixture to synergize, enhance, or otherwise modify the properties of the imaging layer. For example, various dyes, spectral sensitizers, or electrical sensitizers such as Lewis acids may be added to the several layers.

Other modifications and ramifications of the present invention will occur to those skilled in the art upon a reading of the present disclosure. These are intended to be included within the scope of the invention.

#### What is claimed is:

1. In an imaging method wherein a cohesively weak photoresponsive imaging layer comprising electrically photosensitive particles dispersed in an insulating binder is sandwiched between two sheets, then exposed to a pattern of actinic electromagnetic radiation and an electric field thereby providing upon separation of the sheets a positive image on one sheet and a negative image on the other, the improvement comprising: treating the electrically photosensitive particles with from about 20% to about 200% by weight of said particles of a material selected from the group consisting of polyisobutylene succinimide and polyisobutylene succinimide derivatives prior to formation of said images.
2. The method of claim 1 wherein said particle treatment comprises ball milling said material with said particles prior to incorporating said particles in said photoresponsive imaging layer.
3. The method of claim 1 wherein said material is a polyisobutylene succinimide derivative.
4. The method of claim 3 wherein said polyisobutylene succinimide derivatives are derived by reacting polyisobutylene succinimide with a compound having a polar group.
5. The method of claim 4 wherein said compound having a polar group is selected from the group consisting of water, polyhydric alcohols, primary amines, secondary amines, and inorganic metal hydroxides.
6. The method of claim 5 wherein said compound having a polar group is a primary amine.
7. The method of claim 6 wherein said primary amine is represented by the formula



70 wherein  $x$  is from 1 to 10.

8. The method of claim 5 wherein said compound having a polar group is an inorganic metal hydroxide.
9. The method of claim 8 wherein said inorganic metal hydroxide is selected from the group consisting of the

## 11

hydroxides of zinc, cadmium, lead, calcium, manganese and cobalt.

10. The method of claim 9 wherein said inorganic metal hydroxide is selected from the group consisting of the hydroxides of zinc and cadmium.

11. The method of claim 1 wherein the material has a number average molecular weight of up to about 10,000.

12. The method of claim 11 wherein the material has a number average molecular weight of up to about 5,000.

13. An improved fracturable photoresponsive imaging layer of the type having electrically photosensitive particles dispersed in a binder and being fracturable under the combined effect of exposure to electromagnetic radiation to which the particles are sensitive and an applied electric field, wherein the improvement comprises:

a material selected from the group consisting of polyisobutenylsuccinic anhydride and polyisobutenylsuccinic anhydride derivatives substantially uniformly dispersed in said binder.

14. The method of treating electrically photosensitive materials to provide a low background imaging characteristic to said materials, comprising:

intimately contacting the electrically photosensitive materials with from about 20% to about 200% by weight of said materials of a treating agent selected from the group consisting of polyisobutenylsuccinic anhydride and polyisobutenylsuccinic anhydride derivatives.

15. The method of claim 14 further including the step of removing said treating agent from intimate contact with said electrically photosensitive materials.

16. The method of claim 14 wherein the step of intimately contacting comprises ball milling.

17. An electrically photosensitive imaging particle having the characteristic of low background imaging, comprising electrically photosensitive imaging material the surface of which has been intimately contacted with from about 20% to about 200%, by weight of said materials of a treating material selected from the group consisting

## 12

of polyisobutenylsuccinic anhydride and polyisobutenylsuccinic anhydride derivatives.

18. The electrically photosensitive particle of claim 17 wherein said treating material is a polyisobutenylsuccinic anhydride derivative.

19. The electrically photosensitive imaging particle of claim 18 wherein said polyisobutenylsuccinic anhydride derivative is derived from the reaction of polyisobutenylsuccinic anhydride with a polar agent selected from the group consisting of water, polyhydric alcohols, primary amines, secondary amines, and inorganic metal hydroxides.

20. The electrically photosensitive imaging particle of claim 19 wherein the polar agent is a primary amine represented by the formula



wherein  $x$  is from 1 to 10.

21. The electrically photosensitive imaging particle of claim 19 wherein the polar agent is an inorganic metal hydroxide selected from the group consisting of the hydroxides of zinc, cadmium, lead, calcium, manganese and cobalt.

22. The electrically photosensitive imaging particle of claim 17 said treating material has a number average molecular weight of up to about 10,000.

23. The electrically photosensitive imaging particle of claim 17 wherein said treating material has a number average molecular weight of up to about 5,000.

## References Cited

## UNITED STATES PATENTS

|    |           |         |        |       |        |
|----|-----------|---------|--------|-------|--------|
| 35 | 3,615,393 | 10/1971 | Krohn  | ----- | 96-1 M |
|    | 3,573,904 | 4/1971  | Clark  | ----- | 96-1 R |
|    | 3,653,889 | 4/1972  | Luebbe | ----- | 96-1 M |

DAVID KLEIN, Primary Examiner

J. L. GOODROW, Assistant Examiner